# EUROPEAN PATENT SPECIFICATION

(11) **EP 3 680 368 B1**
(45) Date of publication and mention of the grant of the patent: **08.01.2025**
(21) Application number: 18854486.0
(22) Date of filing: 26.01.2018
(51) Int. Cl.: D01F 6/38, D01D 5/247, D01D 5/24, D01F 11/06, D02J 13/00, D06M 13/432, D06M 101/28, D01D 5/00

(54) **METHOD FOR PREPARING HOLLOW FIBER COMPOSITE**
VERFAHREN ZUR HERSTELLUNG VON HOHLFASERVERBUNDSTOFFEN
PROCÉDÉ DE PRÉPARATION D'UN COMPOSITE À FIBRES CREUSES

(30) Priority: 05.09.2017 KR 20170113516; 21.09.2017 KR 20170121575
(43) Date of publication of application: 15.07.2020
(73) Proprietor: Industry-University Cooperation Foundation Hanyang, Ansan-si, Gyeonggi-do 15588 (KR)
(72) Inventor: LEE, Sunyong, Ansan-si Gyeonggi-do 15588 (KR); KANG, Suhee, Ansan-si Gyeonggi-do 15587 (KR); JANG, Joonyoung, Busan 48091 (KR)
(74) Representative: Dr. Gassner & Partner mbB
(86) International application number: PCT/KR2018/001148
(87) International publication number: WO 2019/050106

(56) References cited:
- KR-A- 20110 105 079
- KR-A- 20150 111 548
- KR-A- 20160 050 926
- KR-A- 20160 078 203
- KR-A- 20170 042 157
- US-A1- 2005 112 052

## Description

### [Technical Field]

The present invention relates to a method for preparing a hollow fiber composite, and more particularly to a method for preparing a hollow fiber composite including heat-treating a polymer fiber provided with a precursor.

### [Background Art]

KR 2011 0105079 A discloses a conventional method for preparing a hollow fiber composite, the method comprising preparing polyacrylonitrile nanofibers; providing a precursor containing aluminum oxide onto the polymer fiber; and heat-treating the polymer fiber provided with the precursor, wherein the precursor is heat-treated to be converted into a catalyst and the polymer fiber is heat-treated to have cavities formed therein.

KR 2017 0042157 A proposes a method for preparing a hollow fiber composite, the method comprising preparing a polymer fiber by electrospinning, wherein the fiber comprises a shell portion comprising a metal precursor and a sulfur salt; heat-treating the polymer fiber provided with the precursor, wherein the precursor is heat-treated to be converted into a catalyst and the polymer fiber is heat-treated to have cavities formed therein.

In general, a nanofiber may be defined as a fibrous material having a diameter of less than 1 µm and may be prepared by various methods such as phase separation, self-assembly, chemical vapor disposition (CVD), electrospinning or the like. However, it is known that the electrospinning is most effective in terms of convenient preparation or mass production and applicability of final products.

The electrospinning is a method for preparing a fibrous material having a diameter of less than 1 µm into a web or three-dimensional non-woven fabric by applying a high-voltage electric field to a polymer solution. The nanofiber prepared as above may be used for purposes such as a filter material for air or water purification, a medical anti-adhesive agent, a dressing material, a wiping cloth, a carbon nanofiber for artificial leather and energy storage, an inorganic nanofiber by organic/inorganic mixed spinning, etc., and thus various nanofiber-related technologies have been developed.

For example, Korean Unexamined Patent Publication No. 10-2011-0110643 (Application No.: 10-2010-0030090 and applicant: University-Industry Cooperation Group of Kyung Hee University) discloses a method for preparing a metal-coated nanofiber, including a) preparing an electrospinning solution containing a polymer with a fiber forming ability and an electroless plating catalyst, b) preparing a nanofiber having a diameter of 10 nm to 5 µm by electrospinning the electrospinning solution, and c) electrolessly plating the nanofiber. Besides, various nanofiber-related technologies have been developed now.

### [Disclosure]

### [Technical Problem]

One technical object of the present invention is to provide a method for preparing a hollow fiber composite with an improved surface area.

Another technical object of the present invention is to provide a method for preparing a hollow fiber composite with an improved content of a catalyst.

Still another technical object of the present invention is to provide a method for preparing a hollow fiber composite, which may be applied to various applications.

The technical objects of the present invention are not limited to the above.

### [Technical Solution]

To solve the above technical objects, the present invention provides a method for preparing a hollow fiber composite with the features of claim 1.

According to one embodiment of the invention, the method for preparing a hollow fiber composite includes preparing a polymer fiber, providing a precursor containing nitrogen onto the polymer fiber, and heat-treating the polymer fiber provided with the precursor, in which the precursor is heat-treated to be converted into a catalyst including g-C₃N₄ and the polymer fiber is heat-treated to have cavities formed therein, wherein the polymer fiber provided with the precursor is heat-treated at a temperature of 580°C or above and less than a temperature at which the polymer is carbonized.

According to one embodiment, in the method for preparing a hollow fiber composite, as the polymer fiber provided with the precursor is heat-treated, an adhesive strength between the catalyst and the polymer fiber may be enhanced so that the catalyst may be allowed to fix an outer wall of the polymer fiber, and the polymer fiber may be contracted toward the outer wall from a center of diameter of the polymer fiber so that cavities are formed within the polymer fiber, in which the adhesive strength between the catalyst and the polymer fiber may be stronger than a contraction force of the polymer fiber.

According to one embodiment, the providing of the precursor containing nitrogen onto the polymer fiber may be performed by a method of immersing the polymer fiber into a solution containing the precursor, and the catalyst may be provided onto the polymer fiber in a form of particle or layer depending on a ratio of a weight of the precursor to a weight of the polymer fiber.

According to one embodiment, in the method for preparing a hollow fiber composite, an amount of the precursor permeating into the polymer fiber may be increased as a thickness of the polymer fiber is decreased.

According to one embodiment, the polymer may include polyacrylo nitrile (PAN).

According to one embodiment, the precursor may include urea.

According to another embodiment, the method for preparing a hollow fiber composite may include that an adhesive strength between the catalyst and the polymer fiber is enhanced so that the catalyst is allowed to fix an outer wall of the polymer fiber, and the polymer fiber is contracted toward the outer wall from a center of diameter of the polymer fiber so that the cavities are formed within the polymer fiber.

According to another embodiment, the catalyst may be provided onto the surface of the polymer fiber in a form of particle or layer.

According to another embodiment, the polymer may include polyacrylo nitrile (PAN).

According to another embodiment, the catalyst may be formed prior to the cavities within the polymer fiber.

### [Advantageous Effects]

The method for preparing a hollow fiber composite according to an embodiment of the present invention includes preparing a polymer fiber, providing a precursor containing nitrogen onto the polymer fiber, and heat-treating the polymer fiber provided with the precursor.

Further, as the polymer fiber provided with the precursor is heat-treated, the precursor is converted into a catalyst, and an adhesive strength between the catalyst and the polymer fiber is enhanced, so that the catalyst is allowed to fix an outer wall of the polymer fiber. In this case, the polymer fiber is contracted toward the outer wall from a center of diameter of the polymer fiber, so that cavities are formed within the polymer fiber.

Accordingly, a surface area of the polymer fiber is increased to enhance a content of the catalyst. Further, the hollow fiber composite may be used as an artificial photosynthetic material, a photocatalyst responding to light, etc., depending on a type of the catalyst, and may be also used as a material which carries out reduction of contaminants such as carbon dioxide. Furthermore, the hollow fiber composite may be also used as a composite material, a conductive polymer composite material, a photoelectrochemical water-splitting material, etc., which are used in an electrode material with an improved rate of ionic adsorption, a gas sensor with an improved rate of gas adsorption, an energy storage, and a radiator panel of aircrafts, cars, etc.

### [Description of Drawings]

FIG. 1 is a flowchart for explaining a method for preparing a hollow fiber composite according to an embodiment of the present invention.
FIGS. 2 to 4 are views showing a process of preparing a hollow fiber composite according to an embodiment of the present invention.
FIG. 5 is a view specifically showing a fiber composite formed in a process of preparing a hollow fiber composite according to an embodiment of the present invention.
FIG. 6 is a view for explaining that cavities are formed within a polymer fiber in a process of preparing a hollow fiber composite according to an embodiment of the present invention.
FIG. 7 is a view showing pictures of a hollow fiber composite according to an embodiment of the present invention.
FIG. 8 is a view showing pictures of a nanofiber composite according to Comparative Example 2 of the present invention.
FIGS. 9 to 11 are views showing pictures of hollow fiber composites according to embodiments of the present invention, which are prepared at mutually different temperatures.
FIG. 12 is a graph showing a change in properties of a hollow fiber composite according to an embodiment of the present invention depending on a concentration of urea.

### [Mode for Invention]

Hereinafter, preferred embodiments of the present invention will be described in detail with reference to the accompanying drawings.

When it is mentioned in the specification that one element is on another element, it means that the first element may be directly formed on the second element or a third element may be interposed between the first element and the second element. Further, in the drawings, the thicknesses of the membrane and areas are exaggerated for efficient description of the technical contents.

Further, in the various embodiments of the present invention, the terms such as first, second, and third are used to describe various elements, but the elements are not limited to the terms. The terms are used only to distinguish one element from another element. Accordingly, an element mentioned as a first element in one embodiment may be mentioned as a second element in another embodiment. The embodiments illustrated here include their complementary embodiments. Further, the term "and/or" in the specification is used to include at least one of the elements enumerated in the specification.

In the specification, the terms of a singular form may include plural forms unless otherwise specified. Further, the terms "including" and "having" are used to designate that the features, the numbers, the steps, the elements, or combination thereof described in the specification are present, and may be understood that one or more other features, numbers, step, elements, or combinations thereof may be added.

Further, in the following description of the present invention, a detailed description of known functions and configurations incorporated herein will be omitted when it may make the subject matter of the present invention unnecessarily unclear.

FIG. 1 is a flowchart for explaining a method for preparing a hollow fiber composite according to an embodiment of the present invention, and FIGS. 2 to 4 are views showing a process of preparing a hollow fiber composite according to an embodiment of the present invention.

Referring to FIGS. 1 and 2, a polymer fiber 100 may be prepared (S110). According to one embodiment, the polymer fiber 100 may be prepared by electrospinning a polymer solution. For example, the polymer may include polyacrylo nitrile (PAN). For example, the electrospinning process may be performed through a single nozzle. For example, the polymer fiber 100 may include a PAN nanofiber.

Referring to FIGS. 1 and 3, the precursor 200a may be provided onto the polymer fiber 100 to prepare a fiber composite 300 (S120). According to one embodiment, the precursor 200a may contain nitrogen. For example, the precursor 200a may include urea.

According to one embodiment, the fiber composite 300 may be prepared by a method of immersing the polymer fiber 100 into a solution containing the precursor 200a. For example, if the polymer fiber 100 includes PAN and the precursor 200a includes urea, the fiber composite 300 may be prepared by a method of immersing a PAN fiber having a weight of 50 mg into a solution containing urea having a weight of 3 g.

According to one embodiment, as a thickness of the polymer fiber 100 is decreased, an amount of the precursor 200a permeating into the polymer 100 may be increased. Specifically, if the polymer fiber 100 is immersed into the solution containing the precursor 200a, the precursor 200a may permeate into the polymer fiber 100. In this case, an amount of the precursor 200a permeating into the polymer fiber 100 having a small thickness may be more than an amount of the precursor 200a permeating into the polymer fiber 100 having a large thickness.

Referring to FIGS. 1 and 4, the polymer fiber 100 provided with the precursor 200a may be heat-treated (S130). In other words, the fiber composite 300 may be heat-treated. According to one embodiment, the fiber composite 300 may be disposed within a sintering device 400 and heat-treated. Accordingly, the fiber composite 300 may be subject to sintering.

Hereinafter, as the fiber composite 300 is heat-treated, a process of forming cavities within the polymer fiber 100 will be described with reference to FIGS. 1, 5 and 6.

FIG. 5 is a view specifically showing a fiber composite formed in a process of preparing a hollow fiber composite according to an embodiment of the present invention, and FIG. 6 is a view for explaining that cavities are formed within a polymer fiber in a process of preparing a hollow fiber composite according to an embodiment of the present invention.

Referring to FIGS. 1 and 5, as the fiber composite 300 is heat-treated, the precursor 200a may be converted into a catalyst 200b (S140). In other words, if the fiber composite 300 is heat-treated, the precursor 200a provided onto the polymer fiber 100 may be converted into the catalyst 200b. Accordingly, the catalyst 200b may be provided onto the polymer fiber 100. For example, as described above, if the precursor 200a includes urea, the catalyst 200b may include g-C₃N₄.

According to one embodiment, as shown in (a) of FIG. 5, the catalyst 200b may be provided onto the polymer fiber 100 in a form of particle. According to another embodiment, as shown in (b) of FIG. 5, the catalyst 200b may be provided onto the polymer fiber 100 in a form of layer. Specifically, the catalyst 200b may be provided onto the polymer fiber 100 in a form of particle or layer depending on a ratio of a weight of the precursor 200a to a weight of the polymer fiber 100 in the preparing of the fiber composite 300. For example, the catalyst 200b may be provided onto the polymer fiber 100 in the form of layer, if the polymer fiber 100 includes a PAN fiber and the precursor 200a includes urea, and if a weight ratio between the PAN fiber and the urea exceeds 50 mg : 3 g.

Although (a) and (b) of FIG. 5 show the polymer fiber 100 in a form of cylinder for convenience of explanation, a surface of the polymer fiber 100 may have a concavo-convex shape including concave and convex portions. Accordingly, the catalyst 200b may be provided onto the plurality of concave and convex portions in a form of particle, or may be provided in a form of layer, which conformally covers the surface of the concave and convex portions.

According to one embodiment, the fiber composite 300 may be heat-treated at a temperature of 580 °C or above and less than a temperature at which the polymer is carbonized. The temperature at which the polymer is carbonized may vary depending on a type of the polymer. For example, if the polymer includes PAN, the fiber composite 300 may be heat-treated at a temperature of 580 °C.

In contrast, if the fiber composite 300 is heat-treated at a temperature of less than 580 °C, a contraction of the polymer fiber 100, which will be described below, may not occur, so that cavities may not be easily formed within the polymer fiber 100. Further, if the fiber composite 300 is heat-treated at a temperature, at which the polymer is carbonized, or above, the precursor 200a may not be easily converted into the catalyst 200b, so that cavities may not be easily formed within the polymer fiber 100, which will be described below.

Referring to FIGS. 1 and 6, as the fiber composite 300 is heat-treated, the catalyst 200b may fix an outer wall 100b of the polymer fiber 100 (S150). Specifically, if the fiber composite 300 is heat-treated, adhesion between the catalyst 200b and the polymer fiber 100 may be enhanced, and thus the catalyst 200b may fix the outer wall 100b of the polymer fiber 100.

Further, as the fiber composite 300 is heat-treated, the polymer fiber 100 may be contracted to form cavities 100h within the polymer fiber 100. Specifically, the polymer fiber 100 may be contracted toward the outer wall 100b of the polymer fiber 100 from a center 100a of diameter of the polymer fiber 100. In this case, the adhesive strength between the polymer fiber 100 and the catalyst 200b may be stronger than a contraction force of the polymer fiber 100. Accordingly, the cavities 100h may be formed within the polymer fiber 100.

In other words, if the fiber composite 300 is heat-treated, the precursor 200a provided onto the polymer fiber 100 may be converted into the catalyst 200b and the adhesive strength between the catalyst 200b and the polymer fiber 100 may become strong. Further, as the polymer fiber 100 is heat-treated, a contraction phenomenon of the polymer fiber 100 may occur.

In this case, as the adhesive strength between the polymer fiber 100 and the catalyst 200b is stronger than the contraction force of the polymer fiber 100, the polymer fiber 100 may be contracted while the outer wall 100b of the polymer fiber 100 is fixed by the catalyst 200b. Accordingly, the polymer fiber 100 may be contracted toward the outer wall 100b of the polymer fiber 100 from a center 100a of diameter of the polymer fiber, and the cavities 100h may be formed within the polymer fiber 100.

If the cavities 100h are formed within the polymer fiber 100, the catalyst 200b may be provided not only onto a surface of the polymer fiber 100, but also within the cavities 100h of the polymer fiber 100. However, an amount of the catalyst 200b provided onto the surface of the polymer fiber 100 may be more than an amount of the catalyst 200b provided within the cavities 100h of the polymer fiber 100.

The method for preparing a hollow fiber composite according to an embodiment of the present invention as described above may include preparing the polymer fiber 100, providing the precursor 200a containing nitrogen onto the polymer fiber 100, and heat-treating the polymer fiber 100 provided with the precursor 200a.

Further, as the polymer fiber 100 provided with the precursor 200a is heat-treated, the precursor 200a may be converted into the catalyst 200b, and the adhesive strength between the catalyst 200b and the polymer fiber 100 may be enhanced, so that the catalyst 200b may fix the outer wall 100b of the polymer fiber 100. In this case, the polymer fiber 100 may be contracted toward the outer wall 100b from a center 100a of diameter of the polymer fiber 100, so that the cavities 100h may be formed within the polymer fiber 100.

Accordingly, a surface area of the polymer fiber 100 may be increased to enhance a content of the catalyst 200b. Further, the hollow fiber composite may be used as an artificial photosynthetic material, a photocatalyst responding to light, etc., depending on a type of the catalyst 200b, and may be also used as a material which carries out reduction of contaminants such as carbon dioxide. Furthermore, the hollow fiber composite may be also used as a composite material, a conductive polymer composite material, a photoelectrochemical water-splitting material, etc., which are used in an electrode material with an improved rate of ionic adsorption, a gas sensor with an improved rate of gas adsorption, an energy storage, and a radiator panel of aircrafts, cars, etc.

Hereinafter, specific experimental examples and the results of property evaluation will be described with regard to the hollow fiber composite prepared in accordance with the method for preparing the hollow fiber composite according to an embodiment of the present invention.

### Preparing of hollow fiber composite according to Example

A PAN nanofiber was prepared by electrospinning a polyacrylonitrile (PAN) solution through a single nozzle. After that, a fiber composite was prepared by immersing the PAN nanofiber having a weight of 50 mg into a solution containing urea having a weight of 3 g, after which the fiber composite was heat-treated at a temperature of 580 °C under an atmosphere of argon (Ar) gas, so as to prepare a hollow fiber composite according to an embodiment, in which g-C₃N₄ was provided onto the PAN nanofiber.

### Preparing of nanofiber according to Comparative Example 1

A PAN nanofiber was prepared by electrospinning a PAN solution.

### Preparing of nanofiber composite according to Comparative Example 2

A carbonized PAN nanofiber was prepared by carbonizing a PAN nanofiber which was prepared by electrospinning a PAN solution through a single nozzle. After that, a fiber composite was prepared by immersing the carbonized PAN nanofiber into a solution containing urea and thiourea, after which the fiber composite was heat-treated at a temperature of 580 °C under an atmosphere of argon (Ar) gas, so as to prepare a hollow fiber composite according to an embodiment, in which g-C₃N₄ was provided onto the carbonized PAN nanofiber.

The hollow fiber composite according to the embodiment, the nanofiber according to Comparative Example 1, and the hollow fiber composite according to Comparative Example 2 are summarized in the following Table 1.

**[Table 1]**

| Classification | Structure |
|---|---|
| Example | PAN/g-C₃N₄ hollow fiber composite |
| Comparative Example 1 | PAN nanofiber |
| Comparative Example 2 | Carbonized PAN/g-C₃N₄ nanofiber composite |

FIG. 7 is a view showing pictures of a hollow fiber composite according to an embodiment of the present invention.

Referring to (a) and (b) of FIG. 7, the hollow fiber composite according to the embodiment was photographed through a scanning electron microscope (SEM) with magnification power of 500 nm and 5.00 um. As can be understood from (a) and (b) of FIG. 7, it might be confirmed that the hollow fiber composite according to the embodiment has cavities formed within the fiber composite. Further, the surface area (m²/g) and total pore volume (cm³/g) properties of the hollow fiber composite, which was photographed through the SEM with reference to (a) and (b) of FIG. 7, and the PAN nanofiber according to Comparative Example 1 are summarized in the following Table 2.

**[Table 2]**

| Classification | Surface area (m²/g) (R=coefficient) | | Total pore volume (cm³/g) (p/p₀=0.990) |
|---|---|---|---|
| | a_{s,BET} | aₛ,_{Lang} | |
| Experimental Example | 65.9 (R=0.9999) | No. Lang fit | 0.181 |
| Comparative Example | 19.1 (R=0.9965) | No. Lang fit | 0.015 |

As can be understood from Table 2, it may be seen that the hollow fiber composite according to the embodiment has a surface area value about seven times more than that of the PAN nanofiber, and has a total pore volume value about 12 times more than that of the PAN nanofiber. In other words, it may be seen that the hollow fiber composite according to the embodiment, in which g-C₃N₄ is provided onto the PAN nanofiber, has excellent surface area and total pore volume properties.

FIG. 8 is a view showing pictures of a nanofiber composite according to Comparative Example 2 of the present invention.

Referring to (a) and (b) of FIG. 8, a side and a surface of the nanofiber composite according to above Comparative Example 2 were photographed through a transmission electron microscope (TEM) with magnification power of 50 nm. As can be understood from (a) and (b) of FIG. 8, it may be confirmed that the nanofiber composite according to above Comparative Example 2 does not have cavities formed therein. Further, it may be confirmed that the nanofiber composite according to above Comparative Example 2 has a carbonized PAN surface coated with g-C₃N₄.

FIGS. 9 to 11 are views showing pictures of hollow fiber composites according to embodiments of the present invention, which are prepared at mutually different temperatures.

Referring to FIGS. 9 to 11, the PAN nanofiber according to the embodiment, which was immersed in urea, was heat-treated at temperatures of 300 °C, 400 °C and 580 °C to prepare hollow fiber composites, which were then photographed through the SEM respectively.

As can be confirmed from FIGS. 9 and 10, the hollow fiber composites prepared by being heat-treated at temperatures of 300 °C and 400 °C do not have cavities formed in a part thereof. On the other hand, as can be confirmed from FIG. 11, it might be confirmed that the hollow fiber composite prepared by being heat-treated at a temperature of 580 °C has cavities easily formed therein. Accordingly, in case of preparing the hollow fiber composite according to the embodiment, it may be seen that it is easy to heat-treat the PAN nanofiber immersed in urea at a temperature of 580 °C or above.

FIG. 12 is a graph showing a change in properties of a hollow fiber composite according to an embodiment of the present invention depending on a concentration of urea.

Referring to FIG. 12, in a process of preparing a hollow fiber composite according to the embodiment, a concentration of urea was adjusted in a step of immersing a PAN fiber into a solution containing urea. Next, the hollow fiber composite was prepared when there is no urea (PAN@580) and when there are 2.4 g, 3 g, 4 g and 5 g of urea, after which a transmittance (%)depending on wavenumbers (cm⁻¹) was measured, and the results were shown in a graph of FT-IR (Fourier transform infrared spectroscopy).

As can be understood from FIG. 12, it might be confirmed that the hollow fiber composite (PAN@580) without urea does not show any peak and the hollow fiber composite prepared through immersion into the solution containing 2.4 g of urea shows one peak at 1200-1640 cm⁻¹. On the other hand, it might be confirmed that the hollow fiber composites prepared through immersion into the solutions containing 3 g, 4 g and 5 g of urea show two peaks at 1200-1640 cm⁻¹ and 800-880 cm⁻¹.

In other words, in case of generally measuring FT-IR, a peak related to g-C₃N₄ may be confirmed at 1200-1640 cm⁻¹ and 800-880 cm⁻¹. However, in case of the hollow fiber composites prepared through immersion into the solutions containing 3 g, 4 g and 5 g of urea, it is confirmed that a peak is shown in the range described above. Thus, it may be seen that the hollow fiber composite prepared through immersion into the solutions containing 3 g, 4 g and 5 g of urea have g-C₃N₄ easily formed therein. Accordingly, in case of preparing the hollow fiber composite according to the embodiment, it may be seen that g-C₃N₄ is easily formed by immersing the PAN fiber into the solution containing at least 3 g of urea.

### [Industrial Applicability]

A hollow fiber composite according to an embodiment of the present invention and a method for preparing the same may be utilized in various fields of industry such as a photocatalyst, an artificial photosynthetic material, an electrode material, a gas sensor, an energy storage, a radiator panel, etc.

## Claims

1. A method for preparing a hollow fiber composite (300), the method comprising:
preparing a polymer fiber (100);
providing a precursor (200a) containing nitrogen onto the polymer fiber (100); and
heat-treating the polymer fiber (100) provided with the precursor (200a),
wherein the precursor (200a) is heat-treated to be converted into a catalyst (200b) including g-C₃N₄ and the polymer fiber (100) is heat-treated to have cavities (100h) formed therein,
wherein the polymer fiber (100) provided with the precursor (200a) is heat-treated at a temperature of 580°C or above and less than a temperature at which the polymer is carbonized.

2. The method of claim 1, wherein, as the polymer fiber (100) provided with the precursor (200a) is heat-treated, an adhesive strength between the catalyst (200b) and the polymer fiber (100) is enhanced so that the catalyst (200b) is allowed to fix an outer wall (100b) of the polymer fiber (100), and the polymer fiber (100) is contracted toward the outer wall (100b) from a center (100a) of diameter of the polymer fiber (100) so that cavities (100h) are formed within the polymer fiber (100), and wherein the adhesive strength between the catalyst (200b) and the polymer fiber (100) is stronger than a contraction force of the polymer fiber (100).

3. The method of claim 1, wherein the providing of the precursor (200a) containing nitrogen onto the polymer fiber (100) is performed by immersing the polymer fiber (100) into a solution containing the precursor (200a), and the catalyst (200b) is provided onto the polymer fiber (100) in a form of particle or layer depending on a ratio of a weight of the precursor (200a) to a weight of the polymer fiber (100).

4. The method of claim 1, wherein an amount of the precursor (200a) permeating into the polymer fiber (100) is increased as a thickness of the polymer fiber (100) is decreased.

5. The method of claim 1, wherein the polymer includes polyacrylo nitrile (PAN).

6. The method of claim 1, wherein the precursor (200a) includes urea.

7. The method of claim 1, wherein an adhesive strength between the catalyst (200b) and the polymer fiber (100) is enhanced so that the catalyst (200b) is allowed to fix an outer wall (100b) of the polymer fiber (100), and the polymer fiber (100) is contracted toward the outer wall (100b) from a center (100a) of diameter of the polymer fiber (100) so that the cavities (100h) are formed within the polymer fiber (100).

8. The method of claim 1, wherein the catalyst (200b) is provided onto the surface of the polymer fiber (100) in a form of particle or layer.

9. The method of claim 1, wherein the polymer includes polyacrylo nitrile (PAN).

10. The method of claim 1, wherein the catalyst (200b) is formed prior to the cavities (100h) within the polymer fiber (100) .

## Patentansprüche

1. Verfahren zur Herstellung eines Hohlfaserverbundwerkstoffs (300), wobei das Verfahren umfasst:
Herstellen einer Polymerfaser (100);
Bereitstellen eines Präkursors (200a), der Stickstoff auf der Polymerfaser (100) enthält; und
Wärmebehandlung der mit dem Präkursor (200a) versehenen mit Polymerfaser (100),
wobei der Präkursor (200a) wärmebehandelt wird, um in einen Katalysator (200b) umgewandelt zu werden, der g-C₃N₄ enthält, und wobei die Polymerfaser (100) wärmebehandelt wird, um darin gebildete Hohlräume (100h) aufzuweisen,
wobei die mit dem Präkursor (200a) versehene Polymerfaser (100) bei einer Temperatur von 580 °C oder höher und bei einer geringeren Temperatur als die Temperatur, bei der das Polymer karbonisiert wird, wärmebehandelt wird.

2. Verfahren nach Anspruch 1, wobei sich bei der Wärmebehandlung der mit dem Präkursor (200a) versehenen Polymerfaser (100) die Haftfestigkeit zwischen dem Katalysator (200b) und der Polymerfaser (100) erhöht, so dass der Katalysator (200b) eine Außenwand (100b) der Polymerfaser (100) fixieren kann, und wobei die Polymerfaser (100) von dem Zentrum (100a) des Durchmessers der Polymerfaser (100) in Richtung der Außenwand (100b) kontrahiert wird, so dass Hohlräume (100h) innerhalb der Polymerfaser (100) gebildet werden, und wobei die Haftfestigkeit zwischen dem Katalysator (200b) und der Polymerfaser (100) stärker ist als die Kontraktionskraft der Polymerfaser (100).

3. Verfahren nach Anspruch 1, wobei das Aufbringen des Stickstoff enthaltenden Präkursors (200a) auf die Polymerfaser (100) durch Eintauchen der Polymerfaser (100) in eine den Präkursor (200a) enthaltende Lösung erfolgt und der Katalysator (200b) auf der Polymerfaser (100) in Form von Partikeln oder als Schicht in Abhängigkeit des Verhältnisses des Gewichts des Präkursors (200a) zum Gewicht der Polymerfaser (100) aufgebracht wird.

4. Verfahren nach Anspruch 1, wobei die Menge des Präkursors (200a), der in die Polymerfaser (100) eindringt, mit abnehmender Dicke der Polymerfaser (100) zunimmt.

5. Verfahren nach Anspruch 1, wobei das Polymer Polyacrylnitril (PAN) enthält.

6. Verfahren nach Anspruch 1, wobei der Präkursor (200a) Harnstoff enthält.

7. Verfahren nach Anspruch 1, bei dem die Haftfestigkeit zwischen dem Katalysator (200b) und der Polymerfaser (100) erhöht ist, so dass der Katalysator (200b) eine Außenwand (100b) der Polymerfaser (100) fixieren kann und die Polymerfaser (100) von dem Zentrum (100a) des Durchmessers der Polymerfaser (100) in Richtung der Außenwand (100b) kontrahiert wird, so dass die Hohlräume (100h) innerhalb der Polymerfaser (100) gebildet werden.

8. Verfahren nach Anspruch 1, wobei der Katalysator (200b) auf der Oberfläche der Polymerfaser (100) in Form von Partikeln oder als Schicht bereitgestellt wird.

9. Verfahren nach Anspruch 1, wobei das Polymer Polyacrylnitril (PAN) enthält.

10. Verfahren nach Anspruch 1, wobei der Katalysator (200b) vor den Hohlräumen (100h) innerhalb der Polymerfaser (100) gebildet wird.

## Revendications

1. Procédé de préparation d'un composite à fibres creuses (300), le procédé comprenant :
la préparation d'une fibre polymère (100) ;
la fourniture d'un précurseur (200a) contenant de l'azote sur la fibre polymère (100) ; et
le traitement thermique de la fibre polymère (100) comportant le précurseur (200a),
en ce que le précurseur (200a) est traité thermiquement pour être converti en un catalyseur (200b) comprenant du g-C₃N₄, et la fibre polymère (100) est traitée thermiquement pour former des cavités (100h) à l'intérieur de celle-ci,
en ce que la fibre polymère (100) comportant le précurseur (200a) est traitée thermiquement à une température égale à 580 °C ou supérieure et inférieure à une température à laquelle le polymère est carbonisé.

2. Procédé selon la revendication 1, en ce que lorsque la fibre polymère (100) comportant le précurseur (200a) est traitée thermiquement, une force d'adhésion entre le catalyseur (200b) et la fibre polymère (100) est augmentée de sorte que le catalyseur (200b) peut fixer une paroi extérieure (100b) de la fibre polymère (100), et la fibre polymère (100) est contractée vers la paroi extérieure (100b) à partir d'un centre (100a) de diamètre de la fibre polymère (100) de sorte que des cavités (100h) sont formées à l'intérieur de la fibre polymère (100), et en ce que la force d'adhésion entre le catalyseur (200b) et la fibre polymère (100) est plus forte qu'une force de contraction de la fibre polymère (100).

3. Procédé selon la revendication 1, en ce que la fourniture du précurseur (200a) contenant de l'azote sur la fibre polymère (100) est effectuée en immergeant la fibre polymère (100) dans une solution contenant le précurseur (200a), et le catalyseur (200b) est placé sur la fibre polymère (100) sous forme de particule ou de couche en fonction d'un rapport entre un poids du précurseur (200a) et un poids de la fibre polymère (100).

4. Procédé selon la revendication 1, en ce qu'une quantité du précurseur (200a) imprégnant la fibre polymère (100) augmente au fur et à mesure qu'une épaisseur de la fibre polymère (100) diminue.

5. Procédé selon la revendication 1, en ce que le polymère comprend du polyacrylonitrile (PAN).

6. Procédé selon la revendication 1, en ce que le précurseur (200a) comprend de l'urée.

7. Procédé selon la revendication 1, en ce qu'une force d'adhésion entre le catalyseur (200b) et la fibre polymère (100) est augmentée de sorte que le catalyseur (200b) peut fixer une paroi extérieure (100b) de la fibre polymère (100), et la fibre polymère (100) est contractée vers la paroi extérieure (100b) à partir d'un centre (100a) de diamètre de la fibre polymère (100) de sorte que les cavités (100h) sont formées à l'intérieur de la fibre polymère (100).

8. Procédé selon la revendication 1, en ce que le catalyseur (200b) est fourni sur la surface de la fibre polymère (100) sous forme de particule ou de couche.

9. Procédé selon la revendication 1, en ce que le polymère comprend du polyacrylonitrile (PAN).

10. Procédé selon la revendication 1, **caractérisé en ce que** le catalyseur (200b) est formé avant les cavités (100h) à l'intérieur de la fibre polymère (100).
